

Feb. 17, 1925.

1,526,552

L. KIRSCHBRAUN

PAPER MAKING

Filed Nov. 4, 1921



## UNITED STATES PATENT OFFICE.

LESTER KIRSCHBRAUN, OF CHICAGO, ILLINOIS.

## PAPER MAKING.

Application filed November 4, 1921. Serial No. 512,808.

*To all whom it may concern:*

Be it known that I, LESTER KIRSCHBRAUN, a citizen of the United States, residing in the city of Chicago, county of Cook, and 5 State of Illinois, have invented certain new and useful Improvements in Paper Making, of which the following is a specification.

This invention relates to improvements in paper making, and refers more particularly 10 to the production of a moisture-proof paper, such, for example, as is desired in the manufacture of air-tight or moisture-tight containers.

I have heretofore invented numerous improvements in the art of water-proofing paper, in which an asphaltic or bituminous medium is incorporated in the fibrous stock as the stock is being formed into a web on the usual types of paper-forming machinery. 15

This is accomplished by forming the asphalt into a non-adhesive emulsion of asphalt and water, in which the water forms the external and the asphalt the internal phases respectively of the emulsion.

20 The present invention is not directed specifically to the manner of forming the emulsion in question.

While by means of my prior processes above referred to I have produced water-proof paper which is impervious against water in a liquid phase, there has been more or less tendency for moisture in the form of vapor-laden air to pass through the paper. 25

The object of the present invention is to 30 provide a novel product, process and apparatus for preventing this. It is a further object of the invention to accomplish this result in such a way as to be able to use the usual multi-cylinder machine for making 35 paper in carrying out the process, with such additions as form the novel feature of the present apparatus.

In the present invention, I produce a continuous asphaltic film which is devoid or 40 substantially devoid of any pores through which air can pass.

I have stated that the invention is carried out by making a non-adhesive emulsion of asphalt, clay and water, but an invention 45 can be carried out utilizing my basic idea in which instead of clay and asphalt, other emulsifying agents, as for example soaps, casein, sulfonic acid, salts or other agents may be used, and instead of asphalt 50 other forms of bitumens, hydro-carbons or

pitchy materials may be used—all possessing water-proofing qualities. An invention may be carried out using this basic idea in which the water-proofing constituent may perhaps not necessarily be in a non-adhesive form 60 so long as it is not brought directly into contact with any of the elements of the paper machine which would tend to gum up or interfere with the paper forming operation. 65

To more clearly understand the invention, I have drawn the accompanying drawing, in which Fig. 1 is a somewhat diagrammatic view of a part of a multi-cylinder paper machine, equipped with my invention. 70

Figs. 2 and 3 are diagrammatic plans of the spraying apparatus, by which the asphalt is applied to the fibrous web.

Referring to the drawings, 1 designates a vat containing cylinder mould 2, on which 75 is formed the fibrous web 3, carried by the underside of the blanket 4. 5 designates a second vat, containing the cylinder mould 6, on which is formed a second web 7. 8 and 9 designate couch rolls, 10 the suction 80 box, and 11 a series of press rolls, with which the usual multi-cylinder machine is equipped.

Between the vats 1 and 5 is interposed a spraying device designated as a whole 12, 85 consisting of a series of transversely disposed headers 13, each equipped with a plurality of upwardly extending atomizing nozzles 14. The spraying device is equipped with suitably controlled valves (not shown), whereby any one or more of the manifold 90 nozzles may be used independently of the other.

Above the vat 5 is suitably mounted a transversely disposed manifold 15, containing a plurality of atomizing nozzles 16, the 95 nozzles being inclined upwardly so as to project the asphalt mould into the nipple between the incoming ply and the cylinder mould.

By means of the apparatus shown, the 100 emulsion may be sprayed either through the nozzles 14 across the entire face of the sheet so as to produce a continuous film of any desired thickness, which film is substantially pure asphalt free from a fibre. Also, if 105 desired, an asphalted film may be formed by forcing the non-adhesive emulsion through the nozzles 16; or, if desired, either the nozzles 16 or the nozzles 14 may be used alone. 110

In order to facilitate the retention of the asphalt and to avoid interference with the formation and couching of the sheet, it is desirable to carry the suction in the cylinder moulds as low as possible to produce the driest web capable of retaining the emulsion without disturbance.

I have described the formation of two fibrous webs formed of paper stock only 10 united by a continuous film of non-porous asphalt. However, in some cases it may be desirable to make the webs themselves of asphalted stock, which may be accomplished by mixing the non-adhesive emulsion with 15 the pulp in each vat and between the webs formed of such stock interpose the film of asphalt by means of the spraying devices heretofore described. By using asphalted stock in this manner, the sprayed film of 20 asphalt need not be so heavy, as the absorption of the asphalt into the paper plies is lessened on account of the presence of the asphalted stock.

I claim as my invention:

25. 1. A moisture proof sheet of paper, consisting of a plurality of webs united by means of a film formed of an asphalt and an emulsifying agent.
2. A moisture proof sheet of paper, consisting of a plurality of webs united by means of a film formed of a bituminous substance and an emulsifying agent, said bituminous film being substantially non-porous and devoid of fibrous stock.
35. 3. A process of making a moisture proof sheet, consisting in forming a plurality of fibrous webs, and during such sheet-forming operations, interposing between the webs a moisture proof film of pitchy material.
40. 4. A process of making a moisture proof sheet, consisting in forming a plurality of fibrous webs, and during such sheet-forming operation, interposing between the webs a moisture proof film of pitchy material forming a continuous barrier.
45. 5. A process of making moisture proof paper consisting in forming a plurality of fibrous webs, and applying between the webs a hydrocarbon emulsion in non-adhesive form.
50. 6. A process of making moisture proof paper consisting in forming a plurality of fibrous webs, and simultaneously applying between the webs a hydrocarbon waterproof-

ing agent substantially non-porous and devoid of fibrous stock.

7. A moisture proof sheet of paper consisting of a plurality of webs united by means of a film formed of a flexible fusible waterproof binder and an emulsifying agent. 60

8. A process of making a moistureproof paper consisting in forming a plurality of fibrous webs and applying between the webs a pitchy emulsion in non-adhesive form and subsequently applying heat to coalesce the pitchy substance, and forming a moisture proof barrier. 65

9. A multi-ply sheet having continuous films of pitchy material constituting a moisture proof barrier between the simultaneously formed fibrous plies. 70

10. A moistureproof sheet consisting of a plurality of webs united by a waterproof binder, said binder comprising a film of pitchy material between plies characterized by simultaneous formation. 75

11. A moistureproof sheet consisting of a plurality of webs united by a moistureproof binder, said binder taking the form of a continuous film of pitchy material between the plies and characterized by simultaneous formation. 80

12. The process of making moisture-proof paper which consists in forming a plurality of fibrous webs and applying between the webs a film of pitchy material in an aqueous vehicle. 85

13. A process of making moisture-proof paper consisting in forming a plurality of fibrous webs and simultaneously applying between the webs a pitchy waterproofing agent substantially non-porous and devoid of fibrous stock. 90

14. A moisture-proof paper comprising a plurality of fibrous plies having a barrier of moisture-proof substance interposed therebetween and having the characteristics of having been applied to the wet formation. 95

15. A moisture-proof paper comprising a plurality of fibrous plies, containing a waterproofing substance and a film of substantially fibreless water-proofing substance interposed therebetween, said film having the characteristics of having been applied in an aqueous vehicle to the wet formation. 100 105

LESTER KIRSCHBRAUN.